

# UNITED STATES PATENT OFFICE.

FREDERICK WILLIAM JONES, OF BARWICK, ENGLAND.

## PROCESS OF MAKING EXPLOSIVES.

SPECIFICATION forming part of Letters Patent No. 525,682, dated May 28, 1899.

Application filed March 5, 1897. Serial No. 626,092. (No specimens.)

To all whom it may concern:

Be it known that I, FREDERICK WILLIAM JONES, chemist, a subject of the Queen of Great Britain, residing at Barwick, near Ware, in the county of Herts, England, have invented certain new and useful Improvements in the Manufacture of Explosives, of which the following is a specification.

This invention relates to improvements in the manufacture of explosives which are more especially intended for use with firearms, and has reference more particularly to smokeless or semi-smokeless powders of the kind or class known as "dissolved" or "condensed" powders—that is to say, those containing nitro-cellulose as the principal or one of the principal ingredients and which have been subjected to the action of a suitable solvent or solvents to gelatinize or to dissolve them.

The object of the invention is to enable the densities and rates of combustion of such powders to be regulated or varied, and also to enable a much larger proportion of slowing or "taming" material to be employed than has hitherto been possible without requiring the addition of objectionable metallic nitrates.

Dissolved or condensed powders have usually the objection that the compactness produced by dissolving nitro-cellulose causes the burning to occur only in layers parallel to the original surface, the rate of combustion being comparatively slow, except at high pressures. Consequently to make the powder burn in a gun-barrel very thin grains or laminas must be employed, or the grains must be mechanically perforated at one or more points, so that the burning surfaces do not decrease as the combustion progresses. Furthermore, with such explosives it is impossible to use any larger percentage of what are known as "slowing" or "taming" ingredients without an equally large admixture of an objectionable metallic nitrate. Consequently for some firearms such explosive cannot be used because of the high pressures necessary for their complete combustion. Various attempts have been made to overcome this objection. Some propose to use weak solvents or a method of manufacture that makes a less completely dissolved or

gelatinized product, and others have mixed certain ingredients with the explosive while in a plastic state and extracted them after 55 granulation, making a vesicular grain, while others mix with the nitro-cellulose base large percentages of one or more of the more violent explosives, such as nitro-glycerine, nitro-mannite, methyl nitrate, and explosives 60 of like nature. Now according to my invention I prepare dissolved or condensed smokeless powders by any suitable method and I then submit the powder to one or both of the following processes.

The first process is conducted in what I term the "swelling bath," which consists of an aqueous solution of from twenty per cent. to sixty per cent. of a solvent for the nitro-cellulose used—such as ether, acetone, ketones, and acetic ethers of the paraffins—and in this 70 granulated powder is allowed to soak, with or without agitation and the application of heat, for one or more days. After soaking the solvent is extracted by washing or by passing 75 in steam and condensing the solvent or by some similar process. This bath makes the powder swell and increase in bulk, the amount of increase being greater, the greater the strength of the solution the higher the temperature or the longer the action is continued. It also affects the rate of combustion, so giving a ready means of regulating the density and combustion of any dissolved powder. If any ingredient or ingredients in the granulated powder be soluble in this bath, the 80 bath must first be saturated therewith or the explosive before granulation must have incorporated with it an additional amount of such ingredient or ingredients, so that the 85 bath leaves the desired amount in the finished powder. The powder being freed from its solvent is then dried for use.

The substitute process is only applied to an admixture of the base, mentioned hereinafter, 95 with a solid ingredient or ingredients which will melt below the temperature of boiling water, and when melted have a solvent action on the base, such as the di- and tri- nitro derivatives of benzene, toluene, xylene, and 100 nitro-hydrocarbons of like nature. The dissolved or condensed powder made from such admixtures is granulated in the usual way, and may or may not be treated in the swell-

ing bath. It is then kept in a bath of water at a temperature above the melting-point of the aforementioned ingredient for one or more hours. The effect of this treatment 5 is to make the rate of combustion vary at different points in each grain, and as a consequence the burning surfaces increase as the combustion progresses, which, as will be well understood, enables one to produce an 10 explosive for firearms giving low initial pressures. Also it minimizes the slowing action of the taming ingredient, thus allowing the use of a much larger percentage and the production of an explosive of very low heating 15 properties, owing to the small amount of oxygen present in it. Furthermore, the use of large percentages of these non-volatile substances, which are solvents for nitro-celluloses, lessens the cost of production, as they 20 require very much less volatile solvent to dissolve or gelatinize them when making into grain.

The dissolved or condensed powder which I treat as above may be formed from a base 25 of nitro-cellulose, nitro-hydrocellulose, or nitro-oxycellulose of any degree of nitration, or from any admixture of these with or without nitro-glycerine. With this base I mix, if necessary, one or more nitro-hydrocarbons for 30 regulating or slowing the combustion, such as the nitro- and amido-derivatives of the aromatic series of carbon compounds, picrates, nitro-naphthols, resins, graphite, and such other substances as are now commonly used 35 for this purpose. The composition and granulation of the powder is of course adapted for the purpose intended. The following are, however, three general compositions between the limits of which powders for every kind of 40 firearm can be made by my processes:

First composition: Nitro-cellulose, one hundred per cent. to seventy-five per cent.; slowing material, such as the di- and tri-nitro-benzene, toluene, and xylene, nothing to twenty-five per cent.

Second composition: Nitro-cellulose, ninety per cent. to sixty per cent.; nitro-glycerine, ten per cent. to forty per cent.

Third composition: Nitro-cellulose, ninety 50 per cent. to fifty percent.; nitro-glycerine, ten per cent. to twenty-five per cent.; slowing material, such as the di- and tri-nitro-benzene, toluene, and xylene, nothing to twenty-five per cent.

55 The above ingredients are either mixed together in the wet state and then dried or the dry nitro-cellulose is treated with its solvent containing the other ingredients in solution.

For the usual preliminary dissolving or 60 condensing I prefer to use as a solvent a ketone, preferably either acetone or methyl-ethyl-ketone, owing to the ease with which they can be separated from the explosive and the purity of the resulting product. The 65 amount used depends on the percentage of nitro-glycerine and slowing material in the com-

position, but it varies from sixty to twenty parts, by weight, for every one hundred parts of the original composition. The volatile solvents being mixed with the dried composition 70 by any suitable methods, the whole is left in a vapor-tight vessel for some hours, with or without the application of heat, until the vapors of the solvent have affected the substances to be dissolved, when it is placed in an incorporating and mixing machine and kneaded or worked until the whole is gelatinized. The gelatinized mass is rolled into sheets or forced through dies of definite dimensions and afterward divided into grains or laminae in any 80 suitable manner. The dimensions of the granulated powder will of course vary according to the purpose for which it is made and the energy desired from the explosive. Thus for military purposes a grain or lamina 85 would vary in thickness from 0.015 inch upward, while for sporting-rifles, shotguns, and rim-fire cartridges the thickness would vary from 0.015 inch downward. These granulated products may now be treated by one of 90 the following methods:

First. They may be acted on in the swelling bath, with or without the application of heat, to decrease the density and regulate the combustion. Thus if a granulated powder 95 made of pure nitro-cellulose is heated with a twenty-per-cent. aqueous solution of acetone the powder changes color and swells, so that the density thereof is only two-thirds of the original and the bulk approximates more 100 closely to that of black powder, as a consequence of which it will fill existing cartridges much better than condensed powders that have not been so treated; also, its combustion is so affected that it will burn under 105 very low pressures and can therefore be used in guns where the original powder would be only partially consumed, owing to the high pressures necessary for complete combustion.

Second. If they contain rather large percentages of slowing material or any nitro-glycerine, they may be acted on by the swelling bath only in the cold and the solvent freed from the explosive by washing it with cold water to avoid the extraction of these 115 materials. After extracting the solvent it may be boiled in water to fuse the slowing material and make the rate of combustion vary at different parts of the grain.

Third. Those granulated powders whose 120 density must be as high as possible and which contain ingredients that when fused partially dissolve the base may be kept at a temperature above the melting-point of the aforesaid ingredient for a definite period for the purpose of affecting the combustion of the parts of each grain.

When so treated, comparatively large percentages of slowing or taming ingredients can be used and an explosive of low pressure and low heating properties can therefore be obtained. For instance, if a granulated

dissolved or condensed powder containing twenty per cent. of di- or tri- nitro-benzene, toluene, or xylene be boiled in water for one

solution of a nitro-cellulose solvent, substantially as described.

2. The heroin-described process for pro-

5 or two hours the grains lose their gelatinous appearance and develop entirely different ballistic properties. The fused ingredients not being sufficient to act as solvents on the whole of each grain leave certain parts less acted on and quicker in combustion, the partially-burned grains becoming perforated and the burning surfaces increasing as the combustion progresses.

10 If any of the ingredients are to any extent soluble in water, such as dinitrotoluene, this must be taken into account, so that the correct amount is left in the finished product.

15 In all cases it is desirable to submit the finished product to a washing operation before drying.

20 What I claim is—

1. The heroin-described process for producing a gelatinized smokeless gunpowder of a nitro-cellulose base, which consists in granulating and subsequently swelling the resulting grains by acting on them with an aqueous

25 solution of a nitro-cellulose solvent, substantially as described.

2. The heroin-described process for pro-

30 ducing a gelatinized smokeless gunpowder of a nitro-cellulose base, which consists in granulating and subsequently swelling the resulting grains by acting on them with an aqueous solution of a ketone saturated with any ingredients of the grain soluble therein and afterward washing and drying the same, sub-

35 stantially as described.

3. The process of manufacturing an explosive, which consists in treating a gelatinized condensed powder with an aqueous solution of a ketone previously saturated with any of the ingredients which it would otherwise dissolve out of the powder, substantially as described.

In testimony whereof I have hereunto set my hand this 4th day of February, 1897.

FREDERICK WILLIAM JONES.

Witnesses:

L. G. DUFF GRANT,  
CHAS. B. BURDON.